

# UNITED STATES PATENT OFFICE.

WALTER O. SNELLING, OF ALLENTOWN, PENNSYLVANIA, ASSIGNOR TO TROJAN POWDER COMPANY, OF NEW YORK, N. Y., A CORPORATION OF NEW YORK.

## METHOD OF TREATING UNDRIED ORGANIC NITRATES AND THE LIKE.

1,395,776.

Specification of Letters Patent.

Patented Nov. 1, 1921.

No Drawing. Original application filed March 16, 1920, Serial No. 366,390. Renewed January 21, 1921, Serial No. 439,054. Divided and this application filed March 16, 1921, Serial No. 452,733.

To all whom it may concern:

Be it known that I, WALTER O. SNELLING, a citizen of the United States, and resident of Allentown, Lehigh county, Pennsylvania, 5 have invented certain Improvements in Methods of Treating Undried Organic Nitrates and the like, of which the following is a specification.

My invention relates to the manufacture 10 of explosives and similar materials which, owing to the manufacturing processes employed, are obtained in wet condition, and the object of the invention is to provide a method for reducing the water content of 15 such materials without drying. While my invention may be utilized in the manufacture of a number of materials, I have found it particularly useful as applied to the manufacture of explosives, and for purposes of 20 specific illustration will describe it in connection with such manufacture.

In the manufacture of nitrocellulose, 25 nitrostarch and other solid organic nitrates, said materials, following the nitration and washing processes, are in wet condition, and it has hitherto been the practice to dry them before mixing with other ingredients to produce commercial or military explosives.

Even where it has been desired to produce a 30 wet finished explosive, the preliminary drying process has been deemed necessary because of the undue amount of water present with the organic nitrate following the washing process. While it is manifestly desirable 35 to avoid the drying operation by utilizing the nitrostarch or nitrocellulose in wet condition, as in this way an important item of expense and danger is avoided, experiments have shown that explosives of proper sensi-

40 tiveness cannot be made by the mere mixing of salts with undried nitrostarch or nitrocellulose. For example, nitrostarch after coming from the centrifuge and having its water content reduced therein to the lowest 45 obtainable amount, still contains an average of about 20% of moisture. If now such wet nitrostarch is mixed in equal parts with nitrate of soda or with nitrate of ammonia the completed mix will still contain 10% of 50 moisture, and this is higher than the amount which such a mix can contain and still detonate with certainty with such detonating caps as are commercially used. It is true that by using a smaller amount of the wet

nitrostarch, and a greater amount of the 55 nitrate, mixtures having a lower water content can be obtained. One part of wet nitrostarch may for example be mixed with three parts of sodium nitrate, and in this case if the initial nitrostarch contained 20% of 60 water the final mix will contain but 5% of water. Such a mix is, however, quite as insensitive as the mixture previously described, and which contained 10% of water, 65 for the reason that the amount of nitrostarch has been reduced in proportion as the water has been reduced, the first mixture containing 40% of nitrostarch on a dry basis, and 10% of water, and the second mixture containing 20% of nitrostarch on a 70 dry basis, and 5% of water, and both of these mixtures being relatively insensitive to detonation.

Repeated experiments have shown that there are no proportions in which wet 75 nitrostarch or wet nitrocellulose, after drying to the maximum extent possible in a centrifugal wringer, can be mixed with nitrate of soda or with nitrate of ammonia to form an explosive susceptible to detonation with certainty by the detonators 80 commonly used in commercial work.

I have discovered an inexpensive and convenient method by which sensitive explosives 85 may be obtained from organic nitrates without recourse to the normal drying operation. As an example of my invention, I will describe the method by which I make a nitrostarch explosive from nitrostarch containing 90 25% of water.

I first prepare a concentrated solution of ammonium nitrate and water, preferably using a solution containing about 65% of dissolved ammonium nitrate. I thoroughly mix my wet nitrostarch with such a solution 95 and then apply centrifugal force to remove the excess, thereby substituting a solution of ammonium nitrate for the water which is normally present in the wet material.

As the result of this first stage of my 100 procedure, I obtain instead of nitrostarch wet with 25% of water, nitrostarch which contains 25% of a concentrated solution of ammonium nitrate. As the water originally present in the nitrostarch tends to dilute 105 my original ammonium nitrate solution, in ordinary procedure I obtain an absorbed solution containing about 50% by weight of

ammonium nitrate, and my nitrostarch contains about 25% by weight of this solution, after moderate wringing.

If I now mix equal weights of the nitrostarch so prepared with ammonium nitrate, I obtain a mixture which contains 37.5% of nitrostarch, 56.25% of ammonium nitrate, and 6.25% of water. This mixture is sensitive to commercial detonators, and forms a highly desirable explosive. I may employ 70% of my wet nitrostarch and 30% of ammonium nitrate, and in this case my finished explosive contains 52.5% of nitrostarch, 38.75% of ammonium nitrate, and 8.75% of water, this explosive also being sensitive to a commercial detonating cap.

From the foregoing illustration it will be seen that while the liquid content of the explosive material is not reduced, the water content has been reduced, a portion of the latter being replaced by an ingredient having a function in the finished explosive. Obviously other inorganic oxidizing salts having a high solubility in water may be substituted for ammonium nitrate, such, for example, as calcium nitrate, or ammonium or sodium or potassium chlorate or perchlorate. In the manufacture of some explosives, or other material, the diluting solution need not necessarily be that of a salt performing any function in the finished product other than the diluting function, the method in its broader aspect contemplating the reduction of the water or other liquid content of a wet material by replacement by a concentrated solution of an inorganic salt.

As the solubility of most salts in water is increased by temperature, I obtain a greater drying effect when I use a warm concentrated solution than when I use a cold concentrated solution, since in the former case there is a greater proportion of the solid material in the liquid remaining in the treated material at the close of the process. With materials such as potassium chlorate and potassium perchlorate the use of hot solutions is quite desirable, since these materials are much more soluble in warm water than in cold.

The solid salt which is admixed with the wet organic nitrate prepared as described in this application may or may not be the same material of which a solution is used for diluting the water originally present in the organic nitrate. For example, the water originally present in undried nitrated starch may be replaced by a concentrated solution of ammonium nitrate and the wet nitrostarch so prepared may then be mixed with dry ammonium nitrate or the nitrated starch prepared as described may be mixed with dry sodium nitrate, or with dry ammonium perchlorate or with any other suitable dry salt or mixture of dry salts. In-

stead of a solution of ammonium nitrate or other inorganic salt I may use a concentrated solution of any solid body having high solubility in water.

I do not in this application claim the method which involves substituting for the water in a mixture of a wet inorganic nitrate a solution of a solid body by a displacement process, as said method forms the subject of my application Ser. No. 439,054, of which this is a division.

I claim:

1. The method of treating wet materials to reduce the water content without drying which comprises the step of mixing the material with a concentrated solution of a solid body having high solubility in water, and subsequently removing the excess solution. 80

2. The method of treating wet materials to reduce the water content without drying which comprises the step of thoroughly mixing said wet material with a solution of an inorganic salt and removing by suitable means the excess solution. 85

3. The method of treating wet materials to reduce the water content without drying which comprises the step of thoroughly mixing said wet material with a solution of an inorganic salt and removing by suitable means excess water substantially corresponding in amount to the inorganic salt added. 90 95

4. In the method of manufacturing explosives and the like containing a solid organic nitrate, the step which comprises 100 mixing the undried organic nitrate with a concentrated solution of an inorganic salt, and subsequently removing the excess solution.

5. The method of manufacturing wet explosives containing an organic nitrate and an inorganic salt which comprises mixing a wet organic nitrate with a solution of an inorganic salt, and subsequently removing the excess solution. 105 110

6. The process of making a wet explosive containing a solid organic nitrate and an inorganic salt without drying said organic nitrate, which comprises reducing the amount of water content in said organic nitrate to a required amount by mixing therewith a solution of said inorganic salt, removing excess solution and thereafter adding sufficient of the dry inorganic salt to secure the desired proportion of the several 115 ingredients. 120

7. The method of manufacturing a wet nitrostarch-ammonium nitrate explosive, which comprises mixing undried nitrostarch with a concentrated solution of ammonium nitrate, removing by centrifugal action sufficient liquid to leave in the mass a desired proportion of water, and adding dry ammonium nitrate. 125

WALTER O. SNELLING.